

(No Model.)

W. WILMINGTON.

METHOD OF CASTING CAR WHEELS.

No. 281,422.

Patented July 17, 1883.



WITNESSES:

W. W. Hollingsworth

Edw. C. Byrn.

INVENTOR:

Wm. Wilmington  
BY Maurice L.

ATTORNEYS.

# UNITED STATES PATENT OFFICE.

WILLIAM WILMINGTON, OF TOLEDO, OHIO.

## METHOD OF CASTING CAR-WHEELS.

SPECIFICATION forming part of Letters Patent No. 281,422, dated July 17, 1883.

Application filed June 13, 1883. (No model.)

*To all whom it may concern:*

Be it known that I, WILLIAM WILMINGTON, a citizen of the United States, residing at Toledo, in the county of Lucas and State of Ohio, 5 have invented a new and useful Improvement in Casting Car-Wheels, of which the following is a specification.

This invention is an improvement upon a method of casting car-wheels upon which 10 Letters Patent of the United States have been granted me, No. 273,658, dated March 6, 1883, which patented method consisted in nearly or quite filling a mold for a car-wheel with suitable chill-hardening iron, then immediately 15 placing in the receiving-basin of the mold a small quantity of finely-powdered ferro-manganese or its equivalent, allowing the same to be melted and disseminated through the molten iron in the basin, then pouring a small 20 quantity of molten iron into the basin, causing a partial displacement of the first iron poured out of the mold through proper openings in the same. This method of casting car-wheels produces beneficial results; but it is 25 expensive, because of the waste of metal attending its discharge from the mold and the trouble and cost of caring for the same.

To avoid this expense and lessen the labor in molding the wheel, and still soften the inner parts of the same when casting by an admixture of another quality of metal in the central portions of the wheel, is the object of my improvement.

It consists in nearly or quite filling the mold 35 of any form of a car-wheel with suitable chill-hardening iron. Then immediately after the mold is filled, or when there is a very small space in the same not filled, I place in the central receiving-basin about a pound of ferro-manganese finely powdered, having a large 40 percentage of silicon and carbon in its composition, immediately stirring the same with the molten iron remaining in the basin, causing the metals to combine by fusion, and at intervals inserting a small rod of iron in the openings in the bottom of the basin leading into the mold, and imparting to the rod upward and downward movement, (which experts in casting term "churning.") This will for a 45 short time prevent the molten iron in the openings from being solidified, thereby permitting the melted and disseminated ferro-

manganese in the molten iron in the basin to be diffused downward through the openings in the mold, aided in its downward movement 55 by the churning-rod and the contraction of the molten iron forming the hub, which is incident to bodies of molten metals commencing to cool. The admixture of the ferro-manganese by diffusion and combination with the 60 molten iron at the central parts of the wheel-mold will prevent the same from being too hard and rigid by too sudden cooling when coming in contact with the cold compact cores and moist sand of the mold, thus facilitating 65 the boring of the hub and lessening the liability of the same to fracture when pressing the wheel on the axle. I prefer to use in softening the hub and inner plates of the car-wheels ferro-manganese, because it takes less 70 to produce the desired results. In some qualities of chill-hardening irons I use finely-powdered spiegeleisen in larger quantities instead of the powdered ferro-manganese. In other qualities of chill-hardening cast-iron I use to 75 advantage small particles of cast-iron derived from borings, turnings, drillings, or filings, or otherwise, the same produced from cast-iron made from argillaceous or black-band iron ores. Of these I use still greater proportions in mixing with the chill-hardening iron. In still 80 other qualities of chill-hardening cast-iron I use to soften the hub and inner plates a combination of all or any part of the above-named powdered or small particles of cast-iron ferro-manganese or spiegeleisen in such proportions as practice will show produces the best results. In the use of some of the different qualities of chill-hardening irons I obtain better results by placing the above-named metals in 85 the pouring-ladle, with the molten iron in the same, and allowing it to be melted by contact with the said molten iron in the ladle, then pouring the compound immediately into the basin, and then manipulating the churning-rod, 90 as has been described.

The drawing represents a cross-section of a single-plated car-wheel mold.

A shows the receiving-basin.

B represents two or more openings in the 100 bottom of the basin leading into the mold.

I disclaim as my invention in this application the method of casting car-wheels from two different qualities of molten irons poured

separately into the mold, when the same is melted in separate cupolas or furnaces. I also disclaim the invention of the mold and its apparatus; also the form of the wheel. I furthermore disclaim as my invention all methods of alloying molten iron or steel by an admixture of ferro-manganese, spiegeleisen, or metals made from argillaceous iron ores, when the same is melted in furnace cupola or crucible, for this is common.

I also disclaim as my invention the "churning," as it is termed, of the molten metal leading into molds, for this is common in casting. What I claim as my invention is—

15. The method of casting car-wheels, which

consists in nearly or quite filling the mold of the wheel with suitable chill-hardening cast-iron, then placing in the receiving-basin of the mold finely-powdered ferro-manganese or its equivalent, as described, allowing the same to be melted by the molten iron remaining in the basin, and then agitating the iron remaining in the basin and keeping the inlet-holes open by churning, substantially in the manner and for the purpose heretofore described.

WILLIAM WILMINGTON.

Witnesses:

ALEXANDER WEBER,  
LINCOLN HAYES.